

Aug. 25, 1925.

1,550,957

A. T. GRAHAM

METAL CASTING MOLD

Filed Feb. 12, 1923



INVENTOR

A. T. Graham

By  
Carlos P. Griffin

ATTORNEY

Patented Aug. 25, 1925.

1,550,957

## UNITED STATES PATENT OFFICE.

ARTHUR T. GRAHAM, OF SAN FRANCISCO, CALIFORNIA.

## METAL-CASTING MOLD.

Application filed February 12, 1923. Serial No. 618,647.

*To all whom it may concern:*

Be it known that I, ARTHUR T. GRAHAM, a citizen of the United States, residing at San Francisco, in the county of San Francisco, State of California, have invented a new and useful Metal-Casting Mold, of which the following is a specification in such full and clear terms as will enable those skilled in the art to construct and use the same.

10 This invention relates to a metal casting mold, and its object is to produce sharp castings regardless of the fact that most metals contract slightly at the point of solidification.

15 It will be understood by those skilled in the art that nearly all metals, except antimony, expand considerably upon heating and contract slightly at a more than normal rate of expansion at the point of solidification. This makes it necessary to produce nearly all molds of a size slightly larger than the size the final casting is to be. This disadvantage does not make any great difference where the casting is to be machined to a given size, but in the case of dental work, where it is necessary to produce sharp castings and to use them practically without machining, it is a great disadvantage and necessitates some method of producing castings which will result in a casting as nearly the proper size as it is possible to get it.

20 With the present invention the mold is filled with metallic particles having substantially the same coefficient of expansion under heating as the metal to be cast. These metallic particles are then embedded in a suitable cement so that when the mold is heated it will expand at substantially the same rate as the metal to be cast, and, in the same way, as the metal cools it will contract and thereby produce a sharp casting. The drawing illustrates a mold prepared as described herein for producing a casting.

25 In the drawing the numeral 1 indicates a receptacle for the substance used to produce the mold.

The numeral 2 indicates a plaster-metal-  
30 concrete. The material of which this con-

crete is made is ordinarily, in dental work, a kind of plaster, but in other classes of work it may be simply sand or other fine material in which larger particles of metal, as indicated at 3, are embedded, said particles being large enough in number to substantially fill the mold with the sand and plaster particles, simply filling the voids between the larger particles.

35 As a result of the foregoing method of producing the mold, the coefficient of expansion of the mold is determined by the large number of metal particles contained in it, and which particles are substantially in contact with each other, or at least, sufficiently near in contact with each other to expand the mold at substantially the same rate of expansion as the metal to be cast, whereby the opening in the mold is increased in size, and as the mold cools off, it is reduced in size to its original condition thereby, nearly as may be, producing a sharp casting.

40 In order to prevent the metal particles in the body of the mold from amalgamating with the heated metal to be cast, the metal particles are made of a material which will melt at a slightly higher degree of temperature than the metal casting, and the inside of the mold is coated with a fire-proof paint, as indicated at 4, to prevent the metal to be cast from adhering to the mold.

45 It will be understood by those skilled in the art that the shape of the metal particles is immaterial, the only thing requisite being that they be sufficient in number to give to the mold substantially the same coefficient of expansion under heat as the metal to be cast will have, and that the matrix be sufficient in quantity to hold the mold together properly and capable of withstanding substantially the same high degree of heat as is required to melt the metal for the casting.

50 What I claim is as follows, but modifications may be made in carrying out the invention shown in the drawings as particularly described within the purview of the disclosures:

1. A metal casting mold comprising a

mold made up of granular particles in sufficient number of such a material as to give the mold substantially the same coefficient of expansion and contraction as the metal to be cast.

2. A metal casting mold comprising a mold made up of a body of granular par-

ticles of substantially the same coefficient of expansion as the metal to be cast and a binder for holding said particles together. 10

In testimony whereof I have hereunto set my hand this — day of February A. D. 1923.

ARTHUR T. GRAHAM.